

# UNITED STATES PATENT OFFICE.

SAMUEL SINGLEY, OF NEW YORK, N. Y., ASSIGNOR TO THE MAGNOLIA ANTI-FRICTION METAL COMPANY, OF NEW YORK.

## ANTI-FRICTION ALLOY.

SPECIFICATION forming part of Letters Patent No. 429,158, dated June 3, 1890.

Application filed June 22, 1889. Serial No. 315,249. (Specimens.)

*To all whom it may concern:*

Be it known that I, SAMUEL SINGLEY, of the city, county, and State of New York, have invented a new and Improved Anti-Friction 5 Alloy, of which the following is a specification.

My composition consists of the following metals, in the proportions substantially as stated:

|                |               |         |
|----------------|---------------|---------|
| Lead.....      | 80            | pounds. |
| Antimony.....  | 15            | "       |
| Tin.....       | 5             | "       |
| Bismuth.....   | $\frac{1}{4}$ | "       |
| Aluminium..... | $\frac{1}{4}$ | "       |

15        100 $\frac{1}{2}$ —say 100 pounds. The proportions will vary ten or twenty per cent., depending upon the quality of the lead used. Hard lead will require less of the other ingredients, and soft lead will require more, in 20 proportion to the weight of the lead.

The ingredients are melted and added one by one, care being taken to prevent overheating, and the mass being stirred and skimmed from time to time.

The lead, when molten, I prefer to cleanse 25 by the application of sufficient sal-ammoniac. This I do by adding gradually four to eight ounces of sal-ammoniac, mixing thoroughly, and keeping the molten mass stirred, and removing the scum and dross as it rises; and I 30 also prefer to treat the lead and antimony with sufficient powdered graphite to cover the molten mass, stirring repeatedly, as I have found such treatment to produce better results. If the lead is pure, or has been previously 35 cleansed, the sal-ammoniac may be omitted.

What I claim, and wish to secure by Letters of the United States, is—

The composition of matter to be used for anti-friction purposes, consisting of lead, antimony, tin, bismuth, and aluminium, substantially as described.

SAMUEL SINGLEY.

Witnesses:

CHAS. B. WALLER,  
WALTER K. GRIFFIN.